

## UNITED STATES PATENT OFFICE

2,561,166

## THALLIUM SALTS IN PHOTOGRAPHIC COLOR DEVELOPERS

James E. Bates, Binghamton, N. Y., assignor to  
General Aniline & Film Corporation, New York,  
N. Y., a corporation of Delaware

No Drawing. Application December 1, 1948,  
Serial No. 62,975

7 Claims. (Cl. 95—88)

1

This invention relates to the development of multilayer photographic color emulsions of the negative and reversible color type. It particularly relates to improvements in the color developing solutions and in the process of developing the color negative or color reversal emulsions.

In the commercial practice of developing photographic emulsions where a large quantity of the photographic film is to be developed, it is desirable that all the film be subjected to the developing solution for the same length of time. However, this is rendered difficult because if a number of photographic films have been developed in a given solution, there is a gradual change in tone of the developed film and a loss of developing energy of the solution. Consequently, unless the time of development is increased it is not possible to produce a satisfactory density and contrast. Heretofore it was believed that loss in developing energy of the solution, and consequent increase in time of development was due to depletion of the developing agent and it has been proposed to maintain a relatively uniform development time by replenishing the developer solution. Such replenishment has not been satisfactory as there appears a relatively large shift in development energy of the solution for each portion of film developed for which adequate compensation can be made only by increasing the time of development.

The contrast obtained with a given exposure of film is dependent to a large extent upon the time of development, but a maximum contrast is limited by the maximum gradation of the curve representing density plotted against the logarithm of the time of development. For many purposes a high contrast is desirable as is the case in the development of multi-layer negative color film or multi-layer color film to be developed by the reversal process. In the development of these types of film it is highly desirable to obtain high contrast while at the same time maintaining the time of development as small as possible. In the color development of color film of the negative or reversal type containing color formers in a plurality of layers the shortened development time considerably reduces color fog or stain. It is, therefore, an object of this invention to so improve the color developing solution employed in the color development of photographic negative and reversible type color emulsions as to effect a shortened development time for the same degree of development and consequent reduction in color fog or stain. It is also an object of this invention to produce in color development a color negative film of steeper gradation than can be obtained by modifying the developing time.

2

It has been determined that the addition of soluble thallium salts, such as thallous and thallic nitrate, thallous and thallic sulfate, thallous hydroxide, thallous chloride, thallous bromide and thallous iodide to the color developer for color development of multi-layer photographic color emulsions of the negative and reversal type materially improves the developing characteristics and prolongs the life of the developer.

10 The action of the thallium compounds on the color developer is such that it will effect the revivification of exhausted developer solutions. In applying the invention to the revivifying of such developer solutions, a soluble thallium salt is intermittently added in small increments during the development process. The required amount of the soluble thallium salt may be introduced intermittently after a predetermined quantity of the film has passed through the developing solution or where the film is developed continuously, the soluble thallium salt may be added continuously until the developer is substantially exhausted. If desired, the developer and other ingredients of the developing solution may also be replenished by addition of suitable quantities of developer, preservative and alkali, along with suitable quantities of the soluble thallium salt to maintain the desired properties. In this method of replenishing developer solutions, a relatively small quantity of the soluble thallium salt is used, preferred amounts being about 0.001 to 0.005 gr. per square foot of emulsion developed, depending upon the degree of exhaustion of the developer.

35 In order to obtain the maximum effect on contrast, rate of development and emulsion speed, the soluble thallium salt is added to the fresh developer solution before commencing to develop color negative or color reversal emulsions therein. It has been determined that quantities of thallium salts as small as 0.005 gr. per liter of the color developer solution produced noticeable effects on these color emulsions. Concentrations as high as 0.5 gr. per liter have also been found useful, but the acceleration effect reaches an optimum at from .05 to 0.2 gr. soluble thallium 40 salt per liter of the color developer solution. As compared with my companion application 783-224, filed October 30, 1947, wherein soluble thallium salts are employed in the black and white developer for development of a color reversal film 45 it has been found that somewhat greater amounts of the thallium salt are desirable for use in color developers. Different effects are also produced when the thallium salt is used in the color developer, e. g. color fog or stain is considerably reduced by use of the soluble thallium salts in the 50 55

## 3

color developer for color negative and color reversible film emulsions and in the case of color negative film emulsions the thallium salts in the color developer also produce steeper gradation than can be obtained by any modifications of the development time.

The color developers with which the soluble thallium salts are used may include the usual color developers employed for development of color negative films and for color development of reversible color films of the multi-layer type containing color formers in a plurality of layers. These color developers contain suitable aromatic primary amino developing agents which are characterized by the presence of a free or primary amino group which enables the oxidation product of the developer to couple with the color formers in the film emulsion to form a dye image in the emulsion layer adjacent to the individual particles of the silver image which has been formed by exposure. The primary amino developing agents ordinarily employed are p-phenylene diamines, particularly those having one of the amino groups alkyl substituted. Examples of such developing agents include p-phenylene diamine, monoethyl-p-phenylene diamine, ortho aminodiethyl-aniline, 4,4'-diamino diphenylamine, p-amino dialkyl anilines, such as p-amino-diethyl-aniline and p-amino-dimethyl-aniline. These developing agents are preferably used in the form of their salts such as the hydrochloride since the salts are more soluble and stable than the free base. After the action of the developer has produced a dye image, the silver image may be removed by bleaching in the usual well known manner to leave the color image in the film emulsion.

A suitable developing solution for color development may be prepared as follows:

|                              |          |
|------------------------------|----------|
| P-amino diethyl-aniline HCl  | gr. 2.0  |
| Sodium carbonate (anhydrous) | gr. 50.0 |
| Sodium bisulfite             | gr. 3.0  |
| Potassium bromide            | gr. 0.2  |

are added to sufficient water to make one liter. Hydroxylamine hydrochloride may be added in amounts of approximately 1 gr. to such a developing solution for the color development of color negative emulsions. The ingredients of this typical developer solution may be varied and amounts of the soluble thallium salts, such as thallous nitrate, may be added within the range of from .005 to 0.5 gr. per liter to produce the desirable effects of this invention.

The following examples will serve to further illustrate this invention and the best manner of carrying it out, it being understood that the materials and preparations therein recited are given by way of illustration and not intended as limitations. Unless otherwise specified, the parts are by weight.

## Example 1

A multi-layer negative color film containing dye couplers in a plurality of the individual layers was given normal camera exposure and then processed by the following procedure:

1. Developed 12' at 68° F. with the following color negative developer:

|                                |          |
|--------------------------------|----------|
| P-amino diethyl-aniline HCl    | gr. 3.0  |
| Sodium bisulfite               | gr. 1.0  |
| Sodium carbonate, monohydrated | gr. 60.0 |
| Hydroxylamine HCl              | gr. 1.0  |
| Potassium bromide              | gr. 1.0  |
| Water to make 1.0 l.           |          |

## 4

2. Short stopped 1' in the following solution:

|                      |          |
|----------------------|----------|
| Sodium acetate       | gr. 20.0 |
| Acetic acid          | cc. 10.0 |
| Water to make 1.0 l. |          |

3. Hardened 5' in the following solution:

|                                 |
|---------------------------------|
| Potassium chrome alum, 30.0 gr. |
| Water to make 1.0 l.            |

4. Washed 5' in running water.

5. Bleached 10' in the following solution:

|                                      |          |
|--------------------------------------|----------|
| Mono sodium dipotassium-ferricyanide | gr. 60.0 |
| Potassium bromide                    | gr. 15.0 |
| Disodium phosphate                   | gr. 13.0 |
| Sodium bisulfate                     | gr. 6.0  |
| Water to make 1.0 l.                 |          |

6. Washed 5' in running water.

7. Fixed 5' in the following solution:

|                               |
|-------------------------------|
| Sodium thiosulfate, 200.0 gr. |
| Water to make 1.0 l.          |

8. Washed 10' in running water and dried.

An identically exposed piece of negative color film having the same characteristics as the film treated in the example was given the same processing as above with the exception that 0.05 gr. per liter of thallous nitrate were added to the color negative developer. The same 12' developing time was employed. When the two resultant color negatives were compared photographically, the negative processed with the thallous nitrate displayed  $\frac{1}{2}$  stop more emulsion speed and was considerably steeper in gradation, particularly in the cyan layer, than the normally processed strip.

A third piece of the color negative film was identically exposed and processed through the original set of solutions, except that the development time was increased from 12' to 18' in an attempt to achieve the accelerated developing effects obtained as above by addition of the thallous nitrate. This increase of development time effected an increase in the emulsion speed of  $\frac{1}{2}$  stop, but gave considerably increased fog to the developing colors and did not produce any steepening of the gradation comparable to that produced by the thallium containing developer in the 12' development.

## Example 2

A multi-layer color film of the reversal type containing dye coupling substance in a plurality of the individual layers was given a normal camera exposure and processed by the following procedure:

1. First developed 12' at 68° F. in the following solution:

|                      |          |
|----------------------|----------|
| Metol                | gr. 3.0  |
| Sodium sulfite       | gr. 50.0 |
| Hydroquinone         | gr. 6.0  |
| Sodium carbonate     | gr. 40.0 |
| Sodium thiocyanate   | gr. 2.0  |
| Potassium bromide    | gr. 2.0  |
| Water to make 1.0 l. |          |

2. Rinsed 1' in running water.

3. Hardened 5' in a 3% solution of potassium chrome alum.

4. 2nd exposed to light of photo flood lamp

5. Color developed 16' in the following solution:

P-amino diethyl-aniline HCl gr. 4.0  
 Sodium bisulfite gr. 1.0  
 Sodium carbonate gr. 67.5  
 Potassium bromide gr. 2.5  
 Water to make 1.0 l.

6. Short stopped 2' in the following solution:

Acetic acid cc. 10.0  
 Sodium acetate gr. 20.0  
 Water to make 1.0 l.

7. Hardened 5' in a 3% potassium chrome alum solution.

8. Washed 5'.

9. Bleached 10' in the following solution:

Potassium ferricyanide gr. 60.0  
 Potassium bromide gr. 15.0  
 Dibasic sodium phosphate gr. 13.0  
 Sodium bisulfate gr. 6.0  
 Water to make 1.0 l.

10. Washed 5'.

11. Fixed 5' in 20% hypo solution.

12. Washed 10' and dried.

A similarly exposed piece of color film of the reversal type having the same characteristics as the film treated in this example was processed according to the same procedure, with the exception that 0.5 gr. per liter of thallous nitrate were added to the color developer solution and the color developing time was reduced from 16' to 9'. Substantially the same degree of development was obtained by this shorter development time in the solution containing the thallous nitrate and in addition the highlight stains were reduced perceptibly. No increase in contrast resulted in this instance, but that could not be normally expected with reversal film processing since the final contrast is substantially determined by first development and in this case the accelerator was added to the color developer.

*Example 3*

Additional pieces of reversal type color film having the same characteristics as that used in Example 2 were processed according to the procedure outlined in Example 2, with the exception that the following color developing solution was used:

P-amino dihydroxy-ethyl-aniline sulfate gr. 6.0  
 Sodium bisulfite gr. 1.0  
 Sodium carbonate gr. 100.0  
 Potassium bromide gr. 1.0  
 Water to make 1.0 l.

This color developing agent was found to be much less energetic in its developing energy than the p-aminodiethyl-aniline HCl used in Example 2. Even with a formula of increased strength, as given above, a developing time of 30' was necessary to secure the desired density and color balance. However, upon adding 0.1 gr. per liter of thallous nitrate to this color developer and reducing the color developing time to 15' the same color density and gradation was obtained as in 30' time with the developer containing no thallous nitrate. Also the film developed 15' in the developer containing the thallous nitrate was considerably less stained than the film processed in the normal manner.

*Example 4*

A multi-layer negative color film containing dye couplers in a plurality of the individual lay-

ers was given normal camera exposure and then processed by the following procedure:

1. Developed 12' at 68° F. with the following color negative developer:

P-amino diethyl-aniline HCl gr. 3.0  
 Sodium bisulfite gr. 1.0  
 Sodium carbonate, monohydrated gr. 60.0  
 Hydroxylamine HCl gr. 1.0  
 Potassium bromide gr. 1.0  
 Water to make 1.0 l.

2. Short stopped 1' in the following solution:

Sodium acetate gr. 20.0  
 Acetic acid cc. 10.0  
 Water to make 1.0 l.

3. Hardened 5' in the following solution:

Potassium chrome alum, 30.0 gr.  
 Water to make 1.0 l.

4. Washed 5' in running water.

5. Bleached 10' in the following solution:

Mono sodium dipotassium-ferri-cyanide gr. 60.0  
 Potassium bromide gr. 15.0  
 Disodium phosphate gr. 13.0  
 Sodium bisulfate gr. 6.0  
 Water to make 1.0 l.

6. Washed 5' in running water.

7. Fixed 5' in the following solution:

Sodium thiosulfate, 200.0 gr.  
 Water to make 1.0 l.

8. Washed 10' in running water and dried.

An identically exposed piece of negative color film having the same characteristics as the film treated in the example was given the same processing as above with the exception that 0.100 gr. per liter of thallous iodide were added to the color negative developer. The same 12' developing time was employed. When the two resultant color negatives were compared photographically, the negative processed with the thallous iodide displayed  $\frac{1}{2}$  stop more emulsion speed and was considerably steeper in gradation, particularly in the cyan layer, than the normally processed strip.

A third piece of the color negative film was identically exposed and processed through the original set of solutions, except that the development time was increased from 12' to 18' in an attempt to achieve the accelerated developing effects obtained as above by addition of the thallous iodide. This increase of development time effected an increase in the emulsion speed of  $\frac{1}{2}$  stop, but gave considerably increased fog to the developing colors and did not produce any steepening of the gradation comparable to that produced by the thallium containing developer in the 12' development.

I claim:

1. The method of developing an exposed photographic element having at least one silver halide emulsion layer containing color formers which will couple with the oxidation product of a phenylene diamine developing agent which comprises subjecting such an exposed photographic element to a color developer solution comprising a phenylene diamine developing agent having at least one primary amino group and a soluble thallium salt, the latter being in the concentration of 0.005 to 0.5 gram per liter of solution.

2. The method of claim 1 in which the soluble thallium salt is thallium nitrate.

3. A photographic developer solution for color development of a photographic element having at least one silver halide emulsion layer containing color formers which will couple with the oxidation product of a phenylene diamine developing agent which comprises a phenylene diamine developing agent having at least one primary amino group and a soluble thallium salt, the latter being in the concentration of 0.005 to 0.5 gram per liter of solution.

4. The photographic developer solution of claim 3 wherein the soluble thallium salt is thallium nitrate.

5. A photographic developer solution for color development of a photographic element having at least one silver halide emulsion layer containing color formers which will couple with the oxidation product of a phenylene diamine developing agent which comprises a p-amino diethyl aniline salt and a soluble thallium salt, the latter being in the proportion of 0.005 to 0.5 gram per liter of solution.

6. A photographic developer solution for color development of a photographic element having at least one silver halide emulsion layer containing color formers which will couple with the oxidation product of a phenylene diamine developing agent which comprises a p-amino diethyl aniline salt and a soluble thallium salt, the latter being in the proportion of 0.05 gram per liter of solution.

7. A photographic developer solution for color development of a photographic element having at least one silver halide emulsion layer containing color formers which will couple with the oxidation product of a phenylene diamine developing agent which comprises p-amino diethyl aniline HCl salt and thallous nitrate, the latter being in the proportion of 0.05 gram per liter of solution.

JAMES E. BATES.

#### REFERENCES CITED

The following references are of record in the file of this patent:

#### UNITED STATES PATENTS

Number Name Date  
2,105,274 Steigman Jan. 11, 1938

#### FOREIGN PATENTS

Number Country Date  
477,628 Great Britain Jan. 4, 1937

#### OTHER REFERENCES

Haidrich, Photographische Korrespondenz, Band 73, 1937, pp. 129-134. (Copy in Scientific Library.)

Haidrich, Photographische Korrespondenz, Band 74, 1938, pp. 8-13. (Copy in Scientific Library.)